

## UNITED STATES PATENT OFFICE.

HARRY HOROWITZ, OF NEW YORK, N. Y.

## METHOD OF MAKING SUBSTITUTE FOR LEATHER.

No Drawing.

Application filed February 2, 1927. Serial No. 165,489.

This invention relates generally to material substitutes and has more particular reference to a novel leather or rubber substitute.

- 5 The invention has for an object the provision of an improved leather or rubber substitute of desirable wearing qualities for use in the manufacture of rubber or leather goods, such as soles or heels, of boots or 10 shoes, etc., and which can be manufactured and sold at a low cost.

For further comprehension of the invention, and of the objects and advantages thereof, reference will be had to the following description and to the appended claim in which the various novel features of the invention are more particularly set forth.

The invention consists in the use of 15 chopped or ground leather, with powder, a solution of rubber, raw oil such as raw linseed oil, water, glue, and starch, and to enable others to make use of my invention, I give the following as one of the most approved formulas for compounding and 20 manufacturing the same.

Place in any suitable vessel, one quart of a solution of rubber, preferably made for 25 cheapness, of old or scrap rubber, one ounce of glue, 100 drops of raw oil, one ounce of starch, and 100 to 200% by volume of water. Thoroughly mix these ingredients at a normal 30 temperature. Next, measure out five pounds of ground leather fibres material, and add to it, two ounces of talcum powder, thereafter, thoroughly mix the thus obtained 35 product. Then subject the product to a hydraulic pressure of 25 pounds per square inch for a short period of time, say 10 minutes. Remove the product from the press and 40 manually or mechanically sink the leather fibres from the top and bottom surfaces of the product to a distance of about  $3\frac{1}{2}$ " below these surfaces. This may be accomplished by beating the surfaces with a wire brush, 45 the wires thereof pushing the leather fibres down and as the wires are pulled out, the other material covering the would be apertures caused by the wires. Thereafter subject the product to a hydraulic pressure of about 50 100 pounds per square inch, and form it into a sheet. Repeat the manual or mechan-

ical sinking of the leather fibres from the top and bottom surfaces of the sheet by beating with a wire brush. Finally again subject the product to hydraulic pressure until it is 55 squeezed into a sheet of the desired thickness. Allow the product to dry, which will take about seven days. The product may now be cut as desired, and dyed as desired, and is then in condition for use as a leather or rubber substitute. Due to the sinking of the leather fibres from the surfaces of the sheet, 60 these surfaces are very smooth, and are capable of being highly polished.

While I have illustrated and described my 65 invention with some degree of particularity, I realize that in practice various alterations therein may be made. I therefore reserve the right and privilege of substituting the glue with suitable gum and by changing the 70 form of the details of construction, or otherwise altering the arrangement of the correlated parts without departing from the spirit or the scope of the appended claim.

Having thus described my invention, what 75 I claim as new and desire to secure by United States Letters Patent is:

The method of making a substitute for leather comprising the mixing together of one quart of solution of rubber, one ounce 80 of glue, 100 drops of raw oil, one ounce of starch and 100% to 200% by volume of water at normal temperature, the addition to and thorough incorporation of five pounds of ground leather fibres with the above mixture, the subsequent addition of two ounces of talcum powder, the compressing of the entire mass at a pressure of twenty-five pounds per square inch, the submerging of the leather fibre accumulating on the surfaces of the mass after the above described compression by beating the same with a wire brush, the compressing of the mass at a pressure of one hundred pounds per square inch thereafter, submerging of the leather fibre 85 which is forced to the surface during the second compression step, and the compressing and rolling thereafter required to produce a mass of desired thickness.

In testimony whereof I have affixed my 90 signature.

HARRY HOROWITZ.